# EUROPEAN PATENT SPECIFICATION

(11) **EP 0 136 582 B1**
(45) Date of publication and mention of the grant of the patent: **19.07.1989**
(21) Application number: 84110559.6
(22) Date of filing: 05.09.1984
(51) Int. Cl.: G03C 5/30

(54) **Developer compositions for silver halide photographic materials**
Entwicklerzusammensetzungen für photographische Silberhalogenidmaterialien
Compositions de développement pour matériaux photographiques à l'halogénure d'argent

(30) Priority: 20.09.1983 IT 6521383
(43) Date of publication of application: 10.04.1985
(73) Proprietor: MINNESOTA MINING AND MANUFACTURING COMPANY, St. Paul, Minnesota 55133-3427 (US)
(72) Inventor: Marchesano, Carlo, I-17016 Ferrania/Savona (IT)
(74) Representative: Checcacci, Giorgio

(56) References cited:
- DE-A- 1 772 724
- FR-A- 2 125 325
- GB-A- 1 216 854
- GB-A- 2 010 514
- GB-A- 2 027 920
- RESEARCH DICLOSURE, no. 188, December 1979, pages 692-693, no. 18837, Havant Hampshire, GB; "Use of sequestering agents in black-and-white photographic developers"
- CHEMICAL ABSTRACTS, vol. 91, no. 18, October 1979, page 579, abstract no. 149420u, Columbus, Ohio, US; V.G. BARANOVA et al.: "Silver images from rapid development of cine films", & TEKH. KINO TELEV. 1979, (3), 26-30

## Description

### Field of the invention

The present invention relates to developer compositions for silver halide photographic materials and, particularly, to photographic silver halide developer compositions having improved resistance to aerial oxidation.

### Background of the art

In general, treatment of black and white silver halide photographic materials is carried out in the order of development, stopping, fixing and washing.

Development is ordinarily carried out with alkaline developers containing hydroquinone as a developing agent and alkali metal sulfite as a preservative. Such developers tend to be oxidized by the air during preparation, working and storage. It is a well-known phenomenon that traces of certain metal ions, such as copper and iron, have a catalytic effect on the aerial oxidation of developers (the metal ions may have been introduced as an impurity into the water or into the chemicals used to compound the developing solution).

Some compounds have been proposed to reduce or eliminate the catalytic effect of such metal ions, especially iron, on the aerial oxidation of developers by forming very stable complexes with said metal ions in alkaline solution, but their activity is reduced to a high degree when silver halide photographic materials are treated in continuous transport processing machines, especially at high temperatures. In that case, considerable quantities of air are introduced into developer solutions used in processing machines, this aeration oxidizing more of the developing agent than the real development process itself, causing a rapid degradation of the developer.

GB-A-2,010,514 describes a developer composition for silver halide photographic materials comprising hydroquinone, an alkali metal sulfite, an organic antifogging agent, inorganic alkali agents and an alkanolamine. Research Disclosure (Dec. 1979) N. 188, pages 692-693, describes calcium sequestering agents for use in black and white developers including aminocarboxylic acid compounds, polyphosphonic acid compounds and combinations thereof. GB-A-1,216,854 describes the combined use of a mercapto agent and a benzotriazole agent to maintain the contrast throughout the life of the developer. C.A. Vol. 91 N. 149402u describes a photographic developing-fixing solution containing hydroquinone, Metol, Phenidone, benzotriazole and 1 - phenyl - 5 - mercaptotetrazole.

### Summary of the invention

A developer composition for silver halide photographic materials has been found which has improved resistance to air oxidation, even in the presence of metal ion traces. The composition can be left in continuous transport processing machines for several days, said developer compositions having the following constituents:
(a) hydroquinone or a substituted hydroquinone,
(b) an auxiliary superadditive developing agent,
(c) an alkali metal sulfite,
(d) an organic antifoggant agent,
(e) inorganic alkali agents,
(f) an alkanolamine, and
(g) a sequestering agent selected in the group of diethylenetriaminepentacetic acid (hereinafter referred to as DTPA), 1,3 - diamino - 2 - propanoltetracetic acid (hereinafter referred to as DPTA) and 1 - hydroxyethylidene - 1,1' - diphosphonic acid (hereinafter referred to as HEDP).

### Detailed description of the invention

The present invention relates to a developer composition for silver halide photographic materials comprising hydroquinone or a substituted hydroquinone, an alkali metal sulfite, an organic antifoggant agent and inorganic alkali agents, characterized by further comprising an alkanolamine and a sequestering agent selected in the group of DTPA, DPTA and HEDP.

Preferably, the above described developer composition comprises an additional compound selected in the group of polyphosphates, phosphoric acid, acetic acid, lactic acid and citric acid.

More preferably, the developer composition above comprises an auxiliary developing agent selected from the class of substituted pyrazolidone and p-aminophenol compounds.

Still more preferably, the organic antifoggant agent is selected from the group of mixtures of 5 - nitroindazole and benzimidazole nitrate, 5 - nitrobenzotriazole and 1 - phenyl - 5 - mercaptotetrazole, and benzotriazole and 1 - phenyl - 5 - mercaptotetrazole and the alkanolamine is selected from the group of diethanolamine, triethanolamine, 2 - benzylaminoethanol, 2 - methylaminoethanol, 2 - ethylaminoethanol and 2 - isopropylaminoethanol.

In particular the present invention relates to a developer composition for silver halide photographic materials comprising hydroquinone or a substituted hydroquinone in an amount of 10 to 30 grams per liter, an auxiliary developing agent in an amount of 0.2 to 5 grams per liter, an alkali metal sulfite in an amount of 20 to 50 grams per liter, an organic antifoggant selected in the group of mixtures of 5 - nitroindazole and benzimidazole nitrate, 5 - nitrobenzotriazole and 1 - phenyl - 5 - mercaptotetrazole and benzotriazole and 1 - phenyl - 5 - mercaptotetrazole in an amount of 0.2 to 1.5 grams per liter, inorganic alkali agents sufficient to provide a pH of at least 10 and water sufficient to make up one liter characterized by including:
(a) an alkanolamine in an amount of 5 to 20 grams per liter,
(b) a sequestering agent selected in the group of diethylenetriaminepentacetic acid, 1,3 - diamino - 2 - propanoltetracetic acid and 1 - hydroxyethylene - 1,1' - diphosphonic acid in an amount of 10 to 30 grams per liter, and
(c) a compound selected in the group of polyphosphates, phosphoric acid, acetic acid, lactic acid and citric acid in an amount of 15 to 50 grams per liter.

In another aspect the present invention relates to a single part concentrated developer composition for silver halide photographic materials, to be diluted with water and form a ready for use developer solution, comprising hydroquinone or a substituted hydroquinone, an alkali metal sulfite and inorganic alkali agents, characterized in that it contains an alkanolamine, an organic sequestering agent selected in the group of DTPA, DPTA and HEDP and a mixture of benzotriazole and 1 - phenyl - 5 - mercaptotetrazole antifogging agents.

Preferably, the single part concentrated developer composition above further comprises a compound selected in the group of polyphosphates, phosphoric acid, acetic acid, lactic acid and citric acid.

More preferably the single part concentrated developer composition above comprises an auxiliary developing agent selected from the class of substituted pyrazolidone and para-aminophenol compounds.

In particular the present invention relates to a concentrated developer composition for silver halide photographic materials to be diluted with water to form a ready-for-use developer composition, comprising hydroquinone or a substituted hydroquinone in an amount of 40 to 120 grams per liter, an auxiliary developing agent in an amount of 0.5 to 20 grams per liter, an alkali metal sulfite in an amount of 80 to 200 grams per liter, a mixture of benzotriazole and 1 - phenyl - 5 - mercaptotetrazole antifogging agents in an amount of 0.8 to 6 grams per liter, inorganic alkali agents sufficient to provide a pH of at least 11, and water sufficient to make up 1 liter, characterized by including:
a) an alkalonamine in an amount of 20 to 120 grams per liter,
b) a sequestering agent selected in the group of diethylenetriaminepentacetic acid, 1,3 - diamino - 2 - propanol - tetracetic acid and 1 - hydroxyethylidene - 1,1' - diphosphonic acid in an amount of 20 to 150 grams per liter, and
c) a compound selected in the group of polyphosphates, phosphoric acid, acetic acid, lactic acid and citric acid in an amount of 50 to 150 grams per liter.

The developing agents for silver halide photographic elements suitable for the purposes of the present invention include hydroquinone and substituted hydroquinones (e.g. t - butylhydroquinone, methylhydroquinone, dimethylhydroquinone, chlorohydroquinone, dichlorohydroquinone, bromohydroquinone, 1,4 - dihydroxynaphthalene, methoxyhydroquinone, ethoxyhydroquinone, etc.). Hydroquinone, however, is preferred. Said silver halide developing agents are generally used in an amount from about 5 to 50, preferably 10 to 30 grams per liter of the developing solution.

Such developing agents can be used alone or in combination with auxiliary developing agents which show a superadditive developing effect, such as p-aminophenol and substituted p-aminophenols (e.g. N - methyl - p - aminophenol or metol and 2,4 - diaminophenol) and pyrazolidones (e.g. 1 - phenyl - 3 - pyrazolidone or phenidone) and substituted pyrazolidones (e.g. 4 - methyl - 1 - phenyl - 3 - pyrazolidone and 4,4' - dimethyl - 1 - phenyl - 3 - pyrazolidone). Phenidone, however, is preferred. These auxiliary developing agents are generally used in an amount from about 0.1 to 15, preferably 0.2 to 5 grams per liter of the developer.

The alkali metal sulfites, useful in the developer formulation of this invention as preservatives, include for example sodium and potassium metabisulfite. These are used in an amount from about 15 to 100, preferably 20 to 50 grams per liter of the developer solution.

The organic antifoggant agents, known in the art to eliminate fog on the developed photographic silver halide films, useful in the developer formulations of this invention include derivatives of benzimidazole, benzotriazole, tetrazole, indazole, thiazole, etc. It has been found, however, that particular mixtures of these antifoggant agents are particularly useful in the developer formulations of this invention to assure low fog levels in any working condition and in case of fast silver halide emulsion films having a greater tendency to fog. Such preferred mixtures include mixtures of 5-nitroindazole and benzimidazole nitrate, 5 - nitrobenzotriazole and 1 - phenyl - 5 - mercaptotetrazole and benzotriazole and 1 - phenyl - 5 - mercaptotetrazole. The most preferred combination is benzotriazole and 1 - phenyl - 5 - mercaptotriazole, especially when the developer composition ready for use undergoes a storage prolonged in time, for instance more than 15 days at room temperature, before being used. These mixtures are used in a total amount of from about 0.1 to 3, preferably 0.2 to 1.5 grams per liter of the developer composition. Of course optimum quantities of each compound and proportions can be found by the skilled in the art to respond to specific technical needs. It has been observed, for example, that an excess of 1 - phenyl - 5 - mercaptotetrazole may cause or induce some solarization process especially while developing a color reversal film in a conventional first black-and-white development within a color reversal process. Analogously, an excess of benzotriazole has been found to be related to a decrease of maximum density.

It has been observed, as well, that 5-nitroindazole and benzimidazole give particularly good results when used together in mixtures which contain from 20 to 80 percent (in weight) of one of them with respect to the total mixture. Additionally, benzotriazole and 5 - nitrobenzotriazole have been found to give the best results when used in mixture with 1 - phenyl - 5 - mercaptotetrazole, the latter being present in minor amount with respect to the total mixture, for example in a percent of less than 20 percent, preferably less than 10 percent.

Inorganic alkali agents are used in the developer formulations of this invention to achieve the preferred pH range which is above 10. Such inorganic alkali agents include KOH, NaOH, potassium and sodium carbonate, etc.

Other adjuvants well known in the art can be used in the developer formulation of the present invention, these include restrainers, such as soluble halides (e.g. KBr and NaBr), solvents, buffers (e.g. borates and carbonates), development accelerators, and the like.

In order to be stable to aerial oxidation even during working at high temperatures in continuous transport processing machines, the developer compositions according to the present invention are characterized by the combination of an alkanolamine with the selected sequestering agents above. Alkanolamines suitable for the purpose of the present invention include the hydroxyalkylamines having the general formula: wherein R₁ and R₂ each are a hydrogen atom, an alkyl group having 1 to 3 carbon atoms, a hydroxyalkyl group having 1 to 3 carbon atoms or a benzyl group, R₃ is a hydrogen atom or an alkyl group having 1 to 3 carbon atoms and n is an integer of from 1 to 10.

Preferred alkanolamines include 2 - benzylaminoethanol, ethanolamine, diethanolamine, triethanolamine, choline chloride, 3 - amino - 1 - propanol, 1 - amino - 2 - propanol, 2 - amino - 2 - methyl - 1,3 - propanediol, tris - (hydroxymethyl) - aminopropane, 2 - methylamino - ethanol, 2 - dimethylamino - ethanol, 2 - ethylamino - ethanol, bis - (2 - hydroxypropyl) - amine, 3 - dimethyl- amino - 1 - propanol and 2 - isopropylaminomethanol. Most preferred alkanolamines include the ethanolamines such as diethanolamine, triethanolamine, methylaminoethanol, ethylaminoethanol, isopropylaminoethanol and benzylaminoethanol. The alkanolamines are used in an amount from about 10 to 30, preferably 15 to 20 grams per liter of the developer composition.

The sequestering agents which combined with alkanolamines render the developer composition more stable to aerial oxidation are selected from the group of diethylenetriaminepentacetic acid (DTPA), 1,3 - diamino - 2 - propanoltetracetic acid (DPTA) and 1 - hydroxyethyliden - 1,1' - diphosphonic acid (HEDP). A still more stable combination in addition includes a compound selected from the group of polyphosphates, phosphoric acid, acetic acid, lactic acid and citric acid. The sequestering agents of the former group are used in an amount from about 5 to 50, preferably 10 to 30 grams per liter of the developer solution and the compounds of the latter are used in an amount from about 5 to 100, preferably 15 to 50 grams per liter of the developer solution. Sequestering agents such as ethylenediaminotetracetic acid (EDTA), nitrilotriacetic acid (NTA) and nitrilotrimethylenephosphonic acid (NTPA), having chemical structures similar to those of some compounds of the former group, and compounds such as aminoacetic acid, oxalic acid, glycolic acid, malic acid, aspartic acid, glutammic acid and tartaric acid, having chemical structures similar to those of some compounds of the latter group, used in combination with alkanolamines, did not prove to be as effective as the selected ones in order to prevent developer degradation.

A particular preferred developer formulation will comprise the following ingredients:

Exposed black-and-white silver halide photographic films (e.g. Rapid Access films, X-ray films, Printing Papers, Reversal films) can be satisfactorily processed in machines containing the above reported developer solutions to yield high consistency in terms of sensitometric properties (speed, contrast, fog and maximum density) even if the developer solution is left in the machine processor for several days.

The developer formulation of the present invention may also be prepared from concentrated parts to be diluted with water and from the working solution just prior to its use. Such concentrated parts must be stable in the various storage conditions, problems may arise in making a single concentrated part of the developer solution as such for stability and it is normal practice in the art to divide and package it in two concentrated parts. These parts are combined and diluted with water to the desired strength and placed in the developing tank of the machine.

We have found that the developer formulations of the present invention may be advantageously prepared in a single concentrated part comprising a mixture of benzotriazole and 1 - phenyl - 5 - mercaptotetrazole as antifoggant agent. When such single concentrated part is diluted with water to a working strength, a developer solution is obtained which assures low fog levels in any working conditions. The greater tendency of fast emulsion films to fog when processed at high temperature in continuous transport processing machines has been more effectively countered by said mixture of organic antifoggant agents. Of course, when the developer solution is made by two concentrated parts (a first part comprising the developing agents, the alkali metal sulfite, the alkanolamine and the sequestering agents and a second part comprising the organic antifoggant agents) the choice of such organic antifoggant agents appears not so critical and any mixture of antifoggant agents above described may be used.

A particular preferred concentrated formulation made in a single part according to the present invention will comprise the following ingredients:

The following examples, which further illustrate the present invention, report some experimental data in order to show the stability to aerial oxidation of the developer formulation of the present invention. In particular, the wavelength (in nm) at which the absorption of 100 ml of developer solution stored 3 days in a 1,000 ml conical flask in contact with air became 100% and the variation of pH between fresh and stored developer solution were measured. It is in fact well known that aerial oxidation of alkaline developers containing hydroquinone results in the liberation of alkali (and hence the pH will tend to rise) and in the darkening of the solution. In order to render more critical the aerial oxidation, in some experiments the developer solutions were added with small amounts of iron salts in addition to metal traces that may be present in water or in the chemicals used to compound the solutions. Examples of the present invention indicated with ^{**} have been prepared and/or evaluated together with examples of comparative nature indicated with ^{*.}

### Example 1

Eleven developer solutions for silver halide photographic materials (I to XI) were prepared according to the following Table 1:

The ΔpH (measured at 20°C) and the wavelength values at which the stored solutions have an absorption of 100% (indicated as W₁₀₀) are reported hereinbelow in Table 2 (a longer W₁₀₀ corresponds to a higher degree of oxidation).

The developer solutions containing diethanolamine alone or in combination with EDTA and NTA and the solutions containing DTPA, DPTA, EDTA, NTA and HEDP alone, at the end of the experiment, resulted to be strongly colored and all showed a pH increase higher than 0.5. The solutions containing diethanolamine in combination with DTPA, DPTA and HEDP, on the contrary, resulted to be substantially colorless and showed a pH increase lower than 0.5.

### Example 2

Three photographic developer solutions (XII to XIV) were prepared according to the following Table 3:

ApH at 20°C and W₁₀₀ are reported in Table 4.

The developer solution containing DTPA alone, at the end of the experiment, resulted to be strongly colored and showed a pH increase higher than 0.5. The solutions containing DTPA in combination with diethanolamine or triethanolamine, on the contrary, resulted to be substantially colorless and showed a pH increase lower than 0.5.

### Example 3

Two X-ray developer replenishers (Dev. XV and XVI) suitable for processing X-ray film sheets in automatic processors were prepared according to the following Table 5:

100 ml of each developer were stored for 3 days in a 1,000 ml conical flask in contact with air. ΔpH and W₁₀₀ were then measured. The values are reported hereinbelow in Table 6.

### Example 4

Three developers for rapid access processing machines were prepared according to the following Table 7:

100 ml of each developer were stored in a 1,000 ml conical flask in contact with air. pH at 20°C and W₁₀₀ were then measured at various storage times. Their values are reported hereinbelow in Table 8.

### Example 5

1,000 ml of developers XVII and XVIII were each stored in a 1,500 ml porcelain capsule at room temperature for 3 days.

Samples of various commercially available graphic art films were exposed and processed according to the following processing line:

using both fresh and stored developers.

The sensitometric characteristics of the processed films are reported in the following Table 9.

### Example 6

A liquid concentrated developer (Concentrated Developer XIX), consisting of two parts, was prepared as follows:

A second liquid concentrated developer (Concentrated Developer XX) was prepared in a single part having the components of Parts A and B of Conc. Developer XIX, according to the following composition:

A third liquid concentrated developer (Concentrated Developer XXI), consisting of two parts, was prepared as follows:

A fourth liquid concentrated developer (Concentrated Developer XXII) was prepared in a single part having the components of Parts A and B of Conc. Developer XXI, according to the following composition:

A fifth liquid concentrated developer (Concentrated Developer XXIII) was prepared as follows:

Ten ready-for-use developers were prepared from the above concentrated developers according to the following Table 10:

Sheets of unexposed 3M LOC4 Contact Film were developed in the above described ready-for-use developers for 60" at 35°C, treated in a stop bath comprising 4% acetic acid for 15" at 35°C, fixed in 3M Fix Roll M for 30" at 35°C and finally washed for 5' at 35°C.

The following table (Table 11) reports the minimum density (fog) values of the developed sheets.

### Example 7

Six black-and-white developers were prepared according to the following formula. The sequestering power versus Fe⁺⁺ (tested with (NH₄)₂Fe(S0₄)₂) were measured: the values thereof are reported hereinbelow in Table 12.

### Example 8

Seven developer compositions for rapid access processing machines were prepared according to the following Table 13:

100 ml of each developer were stored at room conditions in a 1,000 ml conical flask in contact with air. ApH after 24 hour storage; absorption Amax after 72 hour storage; time to reach W,ₒₒ=600; and fog of an unexposed 3M LOC4 Film, developed for 60" at 35°C in the above fresh developers (fixed as described in Example 8), were measured. The values are reported in the following Table 14.

The above times to have W,ₒₒ=600 are well sufficient to maintain the stability of the developer solution left in the processing machine without working during interruptions (e.g. during week-ends). Of course, in the normal working conditions a much longer stability of the developer solution (e.g. one or two months) is secured by the replenishment operation; said stability results in any case higher in the presence of the combination of the alkanolamines and the selected sequestering agents according to the present invention.

## Claims

1. A developer composition for silver halide photographic materials comprising hydroquinone or a substituted hydroquinone, an alkali metal sulfite, an organic antifogging agent and inorganic alkali agents, characterized in that said developer composition comprises an alkanolamine and a sequestering agent selected in the group of diethylenetriaminepentacetic acid, 1,3 - diamino - 2 - propanoltetracetic acid and 1 - hydroxyethylidene - 1,1' - diphosphonic acid.

2. The developer composition for silver halide photographic materials according to claim 1 further comprising a compound selected in the group of polyphosphates, phosphoric acid, acetic acid, lactic acid and citric acid.

3. The developer composition for silver halide photographic materials according to claim 1 further comprising an auxiliary developing agent selected in the class of substituted pyrazolidone and p - aminophenol compounds.

4. The developer composition for silver halide photographic materials according to claim 1, in which the organic antifoggant agent is selected in the group of mixtures of 5 - nitroindazole and benzimidazole nitrate, 5 - nitrobenzotriazole and 1 - phenyl - 5 - mercaptotetrazole, and benzotriazole and 1 - phenyl - 5 - mercaptotetrazole.

5. The developer composition for silver halide photographic materials according to claim 1, in which the alkanolamine is selected in the group of diethanolamine, triethanolamine, 2 - benzylaminoethanol, 2 - methylaminoethanol, 2 - ethylaminoethanol and 2 - isopropylaminoethanol.

6. A developer composition for silver halide photographic materials comprising hydroquinone or a substituted hydroquinone in an amount of 10 to 30 grams per liter, an auxiliary developing agent in an amount of 0.2 to 5 grams per liter, an alkali metal sulfite in an amount of 20 to 50 grams per liter, an organic antifoggant agent selected in the group of mixtures of 5 - nitroindazole and benzimidazole nitrate, 5 - nitrobenzotriazole and 1 - phenyl - 5 - mercaptotetrazole and benzotriazole and 1 - phenyl - 5 - mercaptotetrazole in an amount of 0.2 to 1.5 grams per liter, inorganic alkali agents sufficient to provide a pH of at least 10 and water sufficient to make up one liter characterized by including:
(a) an alkanolamine in an amount of 5 to 20 grams per liter,
(b) a sequestering agent selected in the group of diethylenetriaminepentacetic acid, 1,3 - diamino - 2 - propanoltetracetic acid and 1 - hydroxyethylidene - 1,1' - diphosphonic acid in an amount of 10 to 30 grams per liter, and
(c) a compound selected in the group of polyphosphates, phosphoric acid, acetic acid, lactic acid and citric acid in an amount of 15 to 50 grams per liter.

7. A concentrated developer composition for silver halide photographic materials, to be diluted with water to form a ready-for-use developer composition, comprising hydroquinone or a substituted hydroquinone, an alkali metal sulfite and inorganic alkali agents, characterized in that it contains an alkanolamine, a sequestering agent selected in the group of diethylenetriaminepentacetic acid, 1,3 - diamino - 2 - propanoltetracetic acid and 1 - hydroxyethyliden - 1,1' - diphosphonic acid, and a mixture of benzotriazole and 1 - phenyl - 5 - mercaptotetrazole antifogging agents.

8. The concentrated developer composition for silver halide photographic materials according to claim 7 which comprises a compound selected in the group of polyphosphates, phosphoric acid, acetic acid, latic acid and citric acid.

9. The concentrated developer composition for silver halide photographic materials according to claim 7 which comprises diethanolamine as alkanolamine.

10. The concentrated developer composition for silver halide photographic materials according to claim 7 which comprises an auxiliary developing agent selected in the class of substituted pyrazolidone and p-aminophenol compounds.

11. A concentrated developer composition for silver halide photographic materials to be diluted with water to form a ready-for-use developer composition, comprising hydroquinone or a substituted hydroquinone in an amount of 40 to 120 grams per liter, an auxiliary developing agent in an amount of 0.5 to 20 grams per liter, an alkali metal sulfite in an amount of 80 to 200 grams per liter, a mixture of benzotriazole and 1 - phenyl - 5 - mercaptotetrazole antifogging agents in an amount of 0.8 to 6 grams per liter, inorganic alkali agents sufficient to provide a pH of at least 11, and water sufficient to make up 1 liter, characterized by including:
a) an alkanolamine in an amount of 20 to 120 grams per liter,
b) a sequestering agent selected in the group of diethylenetriaminepentacetic acid, 1,3 - diamino - 2 - propanoltetracetic acid and 1 - hydroxyethylidene - 1,1' - diphosphonic acid in an amount of 20 to 150 grams per liter.
c) a compound selected in the group of polyphosphates, phosphoric acid, acetic acid, lactic acid and citric acid in an amount of 50 to 150 grams per liter.

## Patentansprüche

1. Entwicklerzusammensetzung für photographisches Silberhalogenid-Material, umfassend Hydrochinon oder ein substituiertes Hydrochinon, ein Alkalimetallsulfit, ein organisches Antischleiermittel und anorganische alkalische Mittel, dadurch gekennzeichnet, daß die Entwickler - Zusammensetzung ein Alkanolamin und ein sequestrierendes Agens aus der Gruppe Diäthylentriaminpentaessigsäure, 1,3 - Diamino - 2 - propanoltetraessigsäure und 1 - Hydroxyäthyliden - 1,1' - diphosphonsäure umfaßt.

2. Entwickler - Zusammensetzung für photographisches Silberhalogenid - Material nach Anspruch 1, umfassend ferner eine Verbindung aus der Gruppe Polyphosphate, Phosphorsäure, Essigsäure, Milchsäure und Citronensäure.

3. Entwickler - Zusammensetzung für photographisches Silberhalogenid - Material nach Anspruch 1, umfassend ferner ein Entwicklungs - Hilfsmittel aus der Gruppe der substituierten Pyrazolidone und p - Aminophenol - Verbindungen.

4. Entwickler - Zusammensetzung für photographisches Silberhalogenid - Material nach Anspruch 1, in dem das organische Antischleiermittel aus der Gruppe der Gemische von 5 - Nitroindazol und Benzimidazolnitrat, 5 - Nitrobenzotriazol und 1 - Phenyl - 5 - mercaptotetrazol, und Benzotriazol und 1 - Phenyl - 5 - mercaptotetrazol ausgewählt ist.

5. Entwickler - Zusammensetzung für photographisches Silberhalogenid - Material nach Anspruch 1, in dem das Alkanolamin aus der Gruppe Diäthanolamin, Triäthanolamin, 2 - Benzylaminoäthanol, 2 - Methylaminoäthanol, 2 - Äthylaminoäthanol und 2 - Isopropylaminoäthanol ausgewählt ist.

6. Entwickler - Zusammensetzung für photographisches Silberhalogenid - Material, umfassend Hydrochinon oder ein substituiertes Hydrochinon in einer Menge von 10 bis 30 g/Liter, ein Hilfsentwickler in einer Menge von 0,2 bis 5 g/Liter, ein Alkalimetallsulfit in einer Menge von 20 bis 50 g/Liter, ein organisches Antischleiermittel aus der Gruppe der Gemische von 5 - Nitroindazol und Benzimidazolnitrat, 5 - Nitrobenzotriazol und 1 - Phenyl - 5 - mercaptotetrazol und Benzotriazol und 1 - Phenyl - 5 - mercaptotetrazol in einer Menge von 0,2 bis 1,5 g/Liter, ausreichend anorganisches alkalische Stoffe um einen pH-Wert von mindestens 10 zu ergeben, und ausreichend Wasser, um einen Liter zu ergeben, dadurch gekennzeichnet, daß sie einschließt:
(a) ein Alkanolamin in einer Menge von 5 bis 20 g/Liter,
(b) ein sequestrierendes Agens aus der Gruppe Diäthylentriaminpentaessigsäure, 1,3 - Diamino - 2 - propanoltetraessigsäure und 1 - Hydroxyäthyliden - 1,1' - diphosphonsäure in einer Menge von 10 bis 30 g/Liter und
(c) eine Verbindung aus der Gruppe Polyphosphate, Phosphorsäure, Essigsäure, Milchsäure und Citronensäure in einer Menge von 15 bis 50 g/Liter.

7. Konzentrierte Entwickler - Zusammensetzung für photographisches Silberhalogenid - Material, das mit Wasser zu einer gebrauchsfertigen Entwickler - Zusammensetzung verdünnt werden kann, umfassend Hydrochinon oder ein substituiertes Hydrochinon, ein Alkalimetallsulfit und anorganische alkalische Stoffe, dadurch gekennzeichnet, daß es ein Alkanolamin, ein sequestrierendes Agens aus der Gruppe Diäthylentriaminpentaessigsäure 1,3 - Diamino - 2 - propanoltetraessigsäure und 1 - Hydroxyäthyliden - 1,1' - diphosphonsäure und ein Gemisch aus Benzotriazol und 1 - Phenyl - 5 - mercaptotetrazol als Antischleiermittel enthält.

8. Konzentrierte Entwickler - Zusammensetzung für photographisches Silberhalogenidmaterial nach Anspruch 7, das eine Verbindung aus der Gruppe Polyphosphate, Phosphorsäure, Essigsäure, Milchsäure und Citronensäure umfaßt.

9. Konzentrierte Entwickler - Zusammensetzung für photographisches Silberhalogenidmaterial nach Anspruch 7, welches Diäthanolamin als Alkanolamin umfaßt.

10. Konzentrierte Entwickler-Zusammensetzung für photographisches Silberhalogenid - Material nach Anspruch 7, das ein Hilfsentwickler aus der Gruppe der substituierten Pyrazolidone und p - Aminophenolverbindungen umfaßt.

11. Konzentrierte Entwickler - Zusammensetzung für photographisches Silberhalogenid - Material, die mit Wasser zu einer gebrauchsfertigen Entwickler - Zusammensetzung verdünnt werden kann, umfassend Hydrochinon oder ein substituiertes Hydrochinon in einer Menge von 40 bis 120 g/Liter, einen Hilfsentwickler in einer Menge von 0,5 bis 20 g/Liter, ein Alkalimetallsulfit in einer Menge von 80 bis 200 g/Liter, ein Gemisch aus Benzotriazol und 1 - Phenyl - 5 - mercaptotetrazol als Antischleiermittel in einer Menge von 0,8 bis 6 g/Liter, ausreichend anorganische alkalische Stoffe um einen pH-Wert von mindestens 11 zu ergeben, und ausreichend Wasser, um 1 Liter zu erreichen, dadurch gekennzeichnet, daß sie einschließt:
(a) ein Alkanolamin in einer Menge von 20 bis 120 g/Liter,
(b) ein sequestrierendes Agens aus der Gruppe Diäthylentriaminpentaessigsäure, 1,3 - Diamino - 2 - propanoltetraessigsäure und 1 - Hydroxyäthyliden - 1,1' - diphosphonsäure in einer Menge von 20 bis 150 g/Liter,
(c) eine Verbindung aus der Gruppe Polyphosphate, Phosphorsäure, Essigsäure, Milchsäure und Citronensäure in einer Menge von 50 bis 150 g/Liter.

## Revendications

1. Composition de développement pour matériels photographiques à halogénure d'argent, comprenant de l'hydroquinone ou une hydroquinone substituée, un sulfite de métal alcalin, un agent antivoile organique et des agents alcalins inorganiques, caractérisée en ce que cette composition de développement comprend une alcanolamine et un agent séquestrant choisi dans le groupe comprenant l'acide diéthylènetriaminepentacétique, l'acide 1,3 - diamino - 2 - propanoltétracétique et l'acide 1 - hydroxyéthylidène - 1,1' - diphosphonique.

2. Composition de développement pour matériels photographiques à halogénure d'argent suivant la revendication 1, caractérisée en ce qu'elle comprend en outre un composé choisi dans le groupe comprenant des polyphosphates, l'acide phosphorique, l'acide acétique, l'acide lactique et l'acide citrique.

3. Composition de développement pour matériels photographiques à halogénure d'argent suivant la revendication 1, caractérisée en ce qu'elle comprend en outre un agent de développement auxiliaire choisi dans la classe des composés substitués de pyrazolidone et de p - aminophénol.

4. Composition de développement pour matériels photographiques à halogénure d'argent suivant la revendication 1, caractérisée en ce que l'agent antivoile organique est choisi dans le groupe comprenant des mélanges de 5 - nitroindazole et de nitrate de benzimidazole, de 5 - nitrobenzotriazole et de 1 - phényl - 5 - mercaptotétrazole, et de benzotriazole et de 1 - phényl - 5 - mercaptotétrazole.

5. Composition de développement pour matériels photographiques à halogénure d'argent suivant la revendication 1, caractérisée en ce que l'alcanolamine est choisie dans le groupe comprenant la diéthanolamine, la triéthanolamine, le 2 - benzylaminoéthanol, le 2 - méthylaminoéthanol, le 2 - éthylaminoéthanol et le 2 - isopropylaminoéthanol.

6. Composition de développement pour matériels photographiques à halogénure d'argent, comprenant de l'hydroquinone ou une hydroquinone substituée en une quantité de 10 à 30 g/I, un agent de développement auxiliaire en une quantité de 0,2 à 5 g/I, un sulfite de métal alcalin en une quantité de 20 à 50 g/I, un agent antivoile organique choisi dans le groupe comprenant des mélanges de 5 - nitroindazole et de nitrate de benzimidazole, de 5 - nitrobenzotriazole et de 1 - phényl - 5 - mercaptotétrazole et de benzotriazole et de 1 - phényl - 5 - mercaptotétrazole en une quantité de 0,2 à 1,5 g/I, des agents alcalins inorganiques et une quantité suffisante pour donner un pH d'au moins 10, et une quantité suffisante d'eau pour faire un litre, caractérisée, en ce qu'elle comprend:
(a) une alcanolamine en une quantité de 5 à 20 g/I,
(b) un agent séquestrant choisi dans le groupe comprenant l'acide diéthylènetriaminepentacétique, l'acide 1,3 - diamino - 2 - propanoltétracétique et l'acide 1 - hydroxyéthylidène - 1,1' - diphosphonique en une quantité de 10 à 30 g/I, et
(c) un composé choisi dans le groupe comprenant les polyphosphates, l'acide phosphorique, l'acide acétique, l'acide lactique et l'acide citrique, en une quantité de 15 à 50 g/I.

7. Composition de développement concentrée pour matériels photographiques à halogénure d'argent, destinée à être diluée avec de l'eau pour former une composition de développement prête à l'utilisation, comprenant de l'hydroquinone ou une hydroquinone substituée, un sulfite de métal alcalin et des agents alcalins inorganiques, caractérisée en ce qu'elle contient une alcanolamine, un agent séquestrant choisi dans le groupe comprenant l'acide diéthylènetriaminepentacétique, l'acide, 1,3 - diamino - 2 - propanoltétracétique et l'acide 1 - hydroxyéthylidène -1,1' - diphosphonique, et un mélange de benzotriazole et de 1 - phényl - 5 - mercaptotétrazole à titre d'agents antivoiles.

8. Composition de développement concentrée pour matériels photographiques à halogénure d'argent suivant la revendication 7, caractérisée en ce qu'elle comprend un composé choisi dans le groupe comprenant les polyphosphates, l'acide phosphorique, l'acide acétique, l'acide lactique et l'acide citrique.

9. Composition de développement concentrée pour matériels photographiques à halogénure d'argent suivant la revendication 7, caractérisée en ce qu'elle comprend de la diéthanolamine à titre d'alcanolamine.

10. Composition de développement concentrée pour matériels photographiques à halogénure d'argent suivant la revendication 7, caractérisée en ce qu'elle comprend un agent de développement auxiliaire choisi dans la classe comprenant des composés substitués de pyrazolidone et de p - aminophénol.

11. Composition de développement concentrée pour matériels photographiques à halogénure d'argent, destinée à être diluée avec de l'eau pour former une composition de développement prête à l'utilisation, comprenant de l'hydroquinone ou une hydroquinone substituée en une quantité de 40 à 129 g/I, un agent de développement auxiliaire en une quantité de 0,5 à 20 g/l, un sulfite de métal alcalin en une quantité de 80 à 200 g/I, un mélange de benzotriazole et de 1 - phényl - 5 - mercaptotétrazole comme agents antivoiles en une quantité de 0,8 à 6 g/I, des agents alcalins inorganiques en une quantité suffisante pour donner un pH d'au moins 11, et une quantité suffisante d'eau pour faire un litre, caractérisée en ce qu'elle comprend:
(a) une alcanolamine en une quantité de 20 à 120 g/l,
(b) un agent séquestrant choisi dans le groupe comprenant l'acide diéthylènetriaminepentacétique, l'acide 1,3 - diamino - 2 - propanoltétracétique et l'acide 1 - hydroxyéthylidène - 1,1' - diphosphonique en une quantité de 20 à 150 g/I,
(c) un composé choisi dans le groupe comprenant les polyphosphates, l'acide phosphorique, l'acide acétique, l'acide lactique et l'acide citrique en une quantité de 50 à 150 g/I.
